

## UNITED STATES PATENT OFFICE.

MARIA SCHOLZ, OF LEICHLINGEN, GERMANY.

## PROCESS FOR DYEING TEXTILE AND LIKE MATERIALS.

No Drawing. Original application filed June 25, 1923, Serial No. 647,759. Divided and this application filed January 17, 1925. Serial No. 3,049.

To all whom it may concern:

Be it known that I, MARIA SCHOLZ, citizen of Germany, residing at Leichlingen, Germany, have invented certain new and useful

5 Improvements in Processes for Dyeing Textile and like Material, of which the following is a specification.

This application is divisional of my co-pending application, Serial No. 647,759, filed

10 June 25, 1923.

My invention has reference to an improvement in the art of dyeing textile and other material, and it relates more particularly to an improvement in the step of fixing the 15 color on the dyed material, and the object of the invention is to materially shorten and cheapen the color fixing operation and improve at the same time the color fastness of the goods.

20 In the prior art the dyestuffs are commonly fixed by subjecting the dyed material to the action of steam within a closed chamber or treating it by the Mather-Platt process. These procedures are time-consuming, expensive, and do not yield an evenly dyed- 25 through material.

My invention broadly consists in subjecting the dyed material for a relatively very short period, generally not over one minute, 30 to the action of a boiling hot saline solution, such as common salt (sodium chloride) or Glauber's salt (sodium sulfate), to which has been added about 10% of acetic acid; or similar salts, which even in strong solution 35 will not affect the dyestuff deposited on the material.

Since the dyeing of porous material is, by general acceptance, based upon the phenomenon that the dye migrates into the fibre, 40 since the latter shows a stronger attraction to the dye than does the dye solution, the astonishing effect of my new procedure undoubtedly is due to the fact that the hot saline bath takes up more or less water from

the dye solution absorbed by the material, 45 and since the fixing material itself does not react dissolvingly on the dyestuff, the latter is forced to migrate into the fibre and settle therein.

The material is passed into the hot saline 50 bathe preferably immediately or soon after coming from the dye bath, when it is still in more or less wet state, and is left therein normally not over one minute. The new process can also be used to advantage for 55 improving goods previously dyed and finished by other processes, to render them still more color-fast. This is of great importance since it permits the use of cheaper 60 grades of dyestuffs with perfect results in the finished products.

The goods are finally washed and after-treated in suitable manner. Goods treated according to my invention are color-fast to 65 all tests to the highest degree.

What I claim is:—

1. In the art of dyeing, the described color fixing step, which consists in relatively quickly passing the dyed material through a hot aqueous saline solution.

2. In the art of dyeing, the described color fixing step, which consists in relatively quickly passing the dyed material through a hot aqueous saline solution in the presence of a relatively small percentage of acetic 75 acid.

3. In the art of dyeing, the described color fixing step, which consists in relatively quickly passing the dyed material through a hot sodium chloride and acetic acid solu- 80 tion.

4. In the art of dyeing, the described color fixing step, which consists in relatively quickly passing the dyed material through a boiling hot saline solution having an ad- 85 mixture of around 10 percent of acetic acid.

MARIA SCHOLZ.